

# United States Patent [19]

Katsuyama et al.

[11] 3,904,419

[45] Sept. 9, 1975

[54] **NON-SILVER SALT PHOTOSENSITIVE MATERIALS**

[75] Inventors: **Harumi Katsuyama, Minami-ashigara; Hisatake Ono, Saitama, Asaka, both of Japan**

[73] Assignee: **Fuji Photo Film Co., Ltd., Minami-ashigara, Japan**

[22] Filed: **May 25, 1973**

[21] Appl. No.: **364,167**

[30] **Foreign Application Priority Data**

May 26, 1972 Japan..... 47-52264

June 8, 1972 Japan..... 47-57105

[52] **U.S. Cl..... 96/90 R; 96/33; 96/48 R**

[51] **Int. Cl.<sup>2</sup>..... G03C 1/52; G03F 7/02**

[58] **Field of Search..... 96/90 R, 33**

[56] **References Cited**

UNITED STATES PATENTS

3,394,395 7/1968 Mattor et al. .... 96/90 R

|           |         |                       |         |
|-----------|---------|-----------------------|---------|
| 3,647,448 | 3/1972  | DeMeyer et al. ....   | 96/90 R |
| 3,745,012 | 7/1973  | Zarebski .....        | 96/90 R |
| 3,753,718 | 8/1973  | Lonczak.....          | 96/90 R |
| 3,773,515 | 11/1973 | Yamashita et al. .... | 96/90 R |

*Primary Examiner—J. Travis Brown  
Attorney, Agent, or Firm—Sughrue, Rothwell, Mion,  
Zinn and Macpeak*

[57] **ABSTRACT**

Photosensitive materials of excellent preservability which are not based upon a silver salt have a photosensitive layer comprising:

1. a haloalkane whose bond dissociation energy is less than 75 Kcal/mole;
2. a furfurylidene acetal compound
3. an optional phenol compound.

The materials can be processed to form printing plates when the phenol compound is present. Such plates and processes are disclosed.

**12 Claims, No Drawings**

## NON-SILVER SALT PHOTOSENSITIVE MATERIALS

### BACKGROUND OF THE INVENTION

#### 1. Field Of The Invention

The present invention relates to non-silver salt photosensitive materials, printing plates made therefrom and to a process for forming such printing plates.

#### 2. Description Of The Prior Art

When furfural is heated under acidic conditions, a waterinsoluble dark substance is formed (described in "Handbuch der Organischen Chemie" (written by Beilstein), Vol. 17, page 274).

When furfural is reacted with a phenol type compound, a dark furfural-phenol resin is formed (described in "Encyclopedia of Polymer Science and Technology", Vol. 7, pages 432-445).

However, when furfural is stored in a light room, it gradually blackens to become a resin, and, therefore, it is difficult to manufacture photographic materials using furfural.

Light sensitive materials utilizing the light sensitivity of a lower haloalkane are known, for example, haloalkane-aromatic amine type photographic media as described in "Light-Sensitive Systems" (written by J. Kosar), Chapter 8, or lower haloalkanefurfurylidene compound-primary aromatic amine type photographic media as described in Japanese Patent 25952/71 and U.S. Pat. No. 3,394,395. In the former, triphenylmethane dyestuffs form color images. In the latter, Stenhouse dyestuffs which are the reaction products of aldehydes derived from the furfurylidene compounds and amines form color images.

The above mentioned aromatic amines are easily oxidized. For example, when they are left in the air, they gradually blacken. Therefore, these aromatic amines are unsuitable for practical use in light-sensitive materials, since they have such defects that they often stain the background of the materials.

### SUMMARY OF THE INVENTION

An object of the present invention is to provide non-silver salt photo-sensitive materials of excellent preservability.

Another object of the present invention is to provide non-silver salt photo-sensitive materials which may form a colored latent image by exposure and may form a colored visible image by heating.

Still another object of the present invention is to provide non-silver salt photo-sensitive materials which may convert the formed latent image to a visible image in a wide range of temperature.

Yet another object of the present invention is to provide novel printing plates and a method of making printing plates.

The inventors made various studies in order to eliminate the drawbacks of the above mentioned conventional non-silver salt photosensitive materials, and at last have found that it is preferred to use furfural resins or furfural-phenol resins as the image forming component, and to use the furfural-phenol resins for printing plate production.

More precisely, the above mentioned objects of the present invention are attained by using a light-sensitive layer containing a light-sensitive haloalkane, preferably of the following formula (I), having a bond dissociation energy of less than 75 Kcal mole. Preferred materials

are those furfurylidene acetal compound of the following formula (IIa) or (IIb):



5

(wherein X represents a halogen atom (where X's may differ from each other) or a hydrogen atom (but all X's cannot be hydrogen atoms), and R represents a hydrogen atom; a halogen atom; an alkyl group having 1-7 carbon atoms; a halogen-substituted-alkyl group having 1-7 carbon atoms; an acyl group; or an acyl group or arylsulfonyl group substituted with a halogen atom, a nitro group or an aryl group). In forming a photosensitive material per se, however, it is preferred that R represents a hydrogen atom, a halogen atom or a halogen-substituted alkyl group having 1-3 carbon atoms;



wherein R<sub>1</sub> and R<sub>2</sub> each represents one or two phenyl groups or one or two aralkyl groups (having 6-9 carbon atoms) (where the phenyl or aryl ring in the aralkyl group can be substituted with a halogen atom or an alkoxy group having 1-3 carbon atoms), or one or two furfuryl groups,



wherein R<sub>3</sub> represents an alkylene group having 2-7 carbon atoms, which can be substituted with a hydroxymethylene group having 1-4 carbon atoms or an imino group, or may be dimerized by a spiro carbon [illustrated by Formula Ic (where R represents H or CH<sub>3</sub>)]. Preferred R<sub>3</sub> groups in both embodiments are those where R<sub>3</sub> represents a methylene chain of 2-3 carbon atoms which can be substituted by an alkyl group of 1-4 carbon atoms, a hydroxymethylene group of 1-4 carbon atoms or an imino group, and which can be dimerized via a spiro-carbon atom as described above.

The light sensitive layer of the present invention preferably contains, in addition to the light-sensitive haloalkane of the above formula (I) and the furfurylidene acetal compound of the above formula (IIa) or (IIb), a phenol type compound of the following formula (IIIa) or (IIIb):





wherein  $n$  is an integer of 1-3, and  $R_4$  represents a hydrogen atom, a halogen atom, an alkyl group of 1-4 carbon atoms, an alkoxy group of 1-4 carbon atoms, a carboxyl group, an alkoxy carbonyl group of 1-12 carbon atoms, a formyl group, a sulfo group ( $SO_3H$ ), an amino group or an acyl group of 1-4 carbon atoms. The amino group is not preferred for the non-silver salt photosensitive material per se.

Printing plates are formed by image-wise exposing an element having a photosensitive layer containing a photosensitive haloalkane, a furfurylidene acetal compound and a phenol compound represented by the above formulae to light, uniformly heating the photosensitive layer and treating the photosensitive layer with a solvent.

The substitution of the  $R_4$  group in the phenol compound has a great effect in that it increases the oleophilic property of image portions of a printing plate.

#### DETAILED DESCRIPTION OF THE INVENTION

The haloalkane represented by the above formula (I) releases a halogeno radical, and this takes out a hydro-

tolylsulfone,  $\alpha,\alpha,\alpha$ -tribromo- $p$ -nitroacetophenone and  $\alpha,\alpha,\alpha$ -dibromo- $p$ -methylacetophenone, etc. Further, halogen containing compounds which form halogen radicals upon exposure to light or form halogeno-acids in the presence of phenol compounds may be used.

In the non-silver salt photosensitive material per se, the following are preferred: carbon tetrabromide, iodoform, carbon tetraiodide, hexachloroethane, hexafluoroethane, 1,2-diiodoethane, bromo-10 triiodomethane, chloro-diiodomethane, etc., which are solid at room temperature, and in particular, carbon tetrabromide and iodoform are preferred.

The furfurylidene compound to be used in the present invention may easily be synthesized by the reaction 15 of furfural and an alcohol.

For instance, difurfurylidene pentaerythritol can be prepared by refluxing 1 mol equivalent of pentaerythritol and 2 mol equivalents of furfural in toluene in the 20 presence of a catalytic amount of  $p$ -toluenesulfonic acid, e.g., 1/1000 mol equivalent to reactants, removing 2 mol equivalents of water from the azeotropic mixture by means of a quantitative water receiver (Distilling Tube Receiver 0 411 Shibata Kagaku Kikai Kogyo) and pouring the reaction mixture into a large amount of water to precipitate the product. All furfurylidene 25 acetal type compounds among the furfurylidene compounds can be synthesized by the above process merely by altering the starting materials.



gen atom from a solvent and the like to form a hydrohalogenic acid. Accordingly, a large amount of acids exist on the image-exposed part as a latent image. On the other hand, the furfurylidene compound is activated in the presence of the thus formed acid which acts as a catalyst to be converted into a image-like furfural resin of black or dark shade.

The haloalkanes used in this embodiment of the present invention include these compounds whose bond dissociation energy (energy to produce the first halogen free-radical) is less than 75 Kcal/mole, preferably those whose bond dissociation energy is less than 70 Kcal/mole. They are described in "Light-Sensitive Systems" by J. Kosar. For example, carbon tetrabromide, iodoform, carbon tetraiodide, hexachloroethane, 1,2-diiodoethane, bromotriidoethane, bromodiidoethane, triiodoethane, triiodopropane, hexabromohexane, hex-

40 iodohexane, hexabromoheptane,  $\alpha,\alpha,\alpha$ -tribromoacetophenone,  $\alpha,\alpha,\alpha$ -trichloroacetophenone,  $\alpha,\alpha,\alpha$ - $p$ -tetrabromoacetophenone,  $\alpha,\alpha,\alpha$ -tribromomethylphenylsulfone,  $\alpha,\alpha,\alpha$ -tribromomethyl- $p$ -50

For example compound Compound 1 can be produced as follows: furfural 2 mols(192g), pentaerythritol 1 mol (136g) and  $p$ -toluene sulfonic acid 0.2g were heated and refluxed in a distilling tube receiver equipped 21 flask provided with a cooling tube, 11 of benzene being used as the solvent. As the reaction proceeded, water appeared in the receiver (described above), the reaction mixture became black, and some precipitation appeared. After the water was frictionally distilled the reaction product was filtered, and the filtrate poured into 3l of ligroin, whereupon flaked crystals appeared. 200 g of yellow crystals (mp. 161°-3°C) of Compound 1 were thus obtained.

In the following examples of the furfurylidene compounds used in the present invention are shown.

55 1.



iodohexane, hexabromoheptane,  $\alpha,\alpha,\alpha$ -tribromoacetophenone,  $\alpha,\alpha,\alpha$ -trichloroacetophenone,  $\alpha,\alpha,\alpha$ - $p$ -tetrabromoacetophenone,  $\alpha,\alpha,\alpha$ -tribromomethylphenylsulfone,  $\alpha,\alpha,\alpha$ -tribromomethyl- $p$ -

65 2. Difurfurylidene pentaerythritol

2.

5



Furfurylidene propylene ether.

3.



Furfurylidene difurfuryl ether.

4.



Furfurylidene 2-methyl-2-furfurylideneimino-1,3-propylene ether.

5.



Furfurylidene tetramethylethylene ether.

6.



Furfurylidene diphenethyl ether.

7.



Furfurylidene dianisyl ether.

8.



Furfurylidene dianisyl ether.

9.



Furfurylidene dibenzhydryl ether.

10.



Furfurylidene bis-(p-chlorobenzyl) ether.

The non-silver salt photo-sensitive materials of the present invention preferably consist of a support and of a light-sensitive layer applied on the said support and containing the above mentioned components. The light-sensitive layer may further contain a film forming binder. In many cases, the said layer preferably con-

tains the binder (especially to form a printing plate, however). The binder may be anyone of the known binders such as nitrocellulose, benzyl cellulose, polycarbonate, polyvinyl acetate, cellulose acetate, cellulose acetate-butylate, cellulose acetatephthalate, polyvinyl chloride, polystyrene, polyester, polymethylmethacrylate, polyvinyl-pyrrolidone, polyvinyl-butylal, polyphenyleneoxide, etc. It is to be noted that the heating range for fixation may vary, depending upon the selection of the binder and the combination thereof. Binders as are used in the printing plate embodiment are preferably resistant to temperatures less than 200°C and do not react with the compounds of the layer.

As earlier indicated, the objects of the present invention may further preferably be attained, by incorporating a phenol type compound of the formula (IIIa) or formula (IIIb) in the above mentioned light-sensitive layer.

The representatives of the phenol type compounds, for example, pyrogallol, methyl gallate, ethyl gallate, n-propyl gallate, isoamyl gallate, lauryl gallate, stearyl gallate, gallic acid, phloroglucinol, 2,4,6-trihydroxytoluene, 2,4,6-trihydroxyacetophenone, 3-methoxycatechol, 3,4-dihydroxy-benzoic acid, 2,5-dihydroxybenzoic acid, 2,6-dihydroxy-3,5-di-tert.butyl benzoic acid, 2,6-dihydroxy-benzaldehyde, 4,5-dihydroxytoluene, resorcinol, 4-chloro-resorcinol, 3,5-dihydroxy-toluene, hydroquinone, p-hydroxybenzene-

5  
10  
15  
20  
25  
When a light-sensitive material containing a dispersion of a halo-alkane and a polyphenol uniformly dispersed in a binder is exposed to light, the same coloring is in fact noticed. However, even if the resulting dye is heated, the material is merely yellowed and faded without being blackened. In view of such phenomena, it is considered that the dye itself does not have any important action in the light-sensitive system of the present invention. In the next place, when a furfurylidene compound is applied to the above mentioned specimen wherein a benzene type dye is formed, and then is heated, only the part wherein the dye is formed is blackened in dark. That is, it is considered as follows: A great amount of acids are formed in the part of the latent image, and thus the furfurylidene compound is converted to furfural due to the catalytic action of the said acid, and afterwards, the furfural beings to react with a phenol compound to form a furfural-phenol resin. The mechanism on the formation of the furfural-phenol resin is as follows, referring to "Kunststoffe" (written by Koschulz) Vol. 23 (1933), page 97: In the first place, a precondensation reaction proceeds between the furfural and the phenol compound, according to the following reaction formula, and the resulting precondensation product is converted under heating to a dark resin or a furfural-phenol resin having a ternary network structure, via the ring cleavage polymerization of the furan ring.



sulfonic acid, p-bromophenol, 1,5-dihydroxynaphthalene, 1,5-dihydroxy-naphthalene, 1,3-dihydroxy-naphthalene, 2,7-dihydroxy-naphthalene-3-sulfonic acid, etc. 2,4-dihydroxy-5-bromobenzoic acid can also be used, but is non-preferred in the non-silver salt photosensitive material per se embodiment.

Due to the use of the phenol type compound, it is possible to extremely increase the image density, which is, however, somewhat insufficient in the layer comprising a halo-alkane and a furfurylidene compound only. This action of the phenol type compound is higher with the increase of the hydroxyl groups therein. From this view-point, the phloroglucinol derivative is in particular preferred. Another merit due to the use of the phenol type compound is that the latent image is colored in yellow, orange or pink tone, depending upon the constitution of the layer. Accordingly, it is possible to change the latent image to a colored one, and thus the photographic materials containing the phenol type compound are preferable to the formation of various kinds of desired images.

The action of the phenol type compound is supposed as follows: It is considered that the halo-alkane and the phenol compound form a benzene type dye via dehydrohalogenation reaction therebetween according to the following reaction formula:

40  
45  
50  
55  
In the light-sensitive materials of the present invention comprising the above mentioned lower halo-alkane, furfurylidene acetal compound and phenol compound, the lower halo-alkane is reacted with the phenol compound by exposure to release a hydrogen halide, and the resulting hydrogen halide acts to hydrolyze the furfurylidene acetal compound to furfural. In the next place, the thus formed furfural is reacted with the phenol compound to form a precondensation product. The resulting precondensation product is then converted by heating to a resin having ternary structure. Accordingly, it is noted that the phenol type compound added to this system acts to serve as a sensitizing agent and as a coloring agent.

55  
60  
65  
The light sensitive materials of the present invention are prepared by dissolving a halo-alkane, a furfurylidene acetal compound and optionally a film forming binder, and further optionally a phenol type compound (the latter two components being used for a printing plate) in an organic solvent (such as toluene, benzene, dioxane, alcohol, tetrahydrofuran, chloroform, methyl-ethylketone, ethyl acetate or the like), and then applying the resulting solution on a support.

60  
65  
For best results, the haloalkane having a dissociation energy of less than 75 kcal/mol, preferably less than 70 Kcal/mol, is present in an amount of from about 0.01



to about 100 g/m<sup>2</sup> of support. Generally, in the printing plate embodiment, it is preferred to use from 0.5 to 10 g/m<sup>2</sup> of support, whereas in the non-silver salt photosensitive material embodiment it is acceptable to use somewhat lesser amounts, i.e., where one merely desires to form an image, and in this case, a preferred amount of haloalkane is from 0.2 to 0.5 g/m<sup>2</sup>. These ranges can, of course, overlap, but, generally speaking lesser amounts will be used in image formation per se and somewhat greater amounts in printing plate formation, where layer removal is mandatory. For best results, per one weight part of haloalkane, the following component weight parts are used: furfurylidene acetal, ca. 0.05 to ca. 50, preferably 0.1-10; phenolic compound, ca. 0.05 to ca. 100 preferably 0.1-20; and film binder ca. 0.03 to ca. 10, preferably 0.1-5. Such a system is easily applied from a solvent in an amount of ca. 10 to ca. 5,000, preferably 50-500, same basis. The above ranges find most special application to the printing plate embodiment.

In the non-silver salt photosensitive material embodiment, however, the weight ratio of the haloalkane to the furfurylidene compound is preferably 0.1-3, better yet 0.5-2, and the weight ratio of the phenol type compound to the furfurylidene compound is preferably 5 or less, better yet 0.05-2. The amount of the binder to be used is not specifically limited, and is sufficient to be able to carry the respective components. However, a preferred ratio by weight of haloalkane to binder is within the range of from about 0.03 to about 10, preferably from 0.1 to 5, weight parts of haloalkane to weight part of binder.

The support may be anyone which has been conventionally used in this field, for example, paper, a plastic film or a metal plate such as aluminum plate or the like. As for the paper support, baryta paper or a paper coated with a high molecular compound (such as polyethylene, polyvinyl alcohol) is in particular preferred.

The thickness of the film coated for the light-sensitive layer is, in general, 0.1-50  $\mu$ , most preferably 1-10  $\mu$  for the non-silver salt embodiment. Excellent results are obtained in the printing plate embodiment when the thickness of the photosensitive layer is about 0.1 to about 30  $\mu$ , better yet 0.5 to 10  $\mu$ .

For printing plate formation, however, the surface of the support should be hydrophilic so as to function as a printing plate. If the support selected is not inherently hydrophilic, the surface of the support can be so rendered by known methods such as chemical treatment, graining, anodizing, the application of a hydrophilic layer thereto, etc.

There is no substantial limitation on the support so long as it is not excessively deformed at the heating conditions used or deteriorated by the solvent used. The degree of hydrophilicity illustrated by the support is not overly important so long as it is generally in accordance with degrees of hydrophilicity used in prior art printing plates.

When an image is formed by using the photosensitive material of the present invention, the said material is exposed image-wise by means of a light of 3000-6000  $\text{\AA}$  wavelength and then is heated at a temperature ranging from room temperature to 200°C. Preferred heating conditions are within a range of from about 50° to about 150°C for about 30 seconds to 5 minutes. The heating is performed for the purpose of the resin formation (that is, reaction acceleration) and of the removal of the remaining halo-alkanes (that is, fixation), and the time for the heating may freely be de-

termined. As the case may be, even though the heating step is omitted, a permanent image can be formed.

In the printing plate embodiment, the photosensitive material of the present invention is image-wise exposed to light of a wavelength of about 3000 to preferably 5000  $\text{\AA}$ . Electromagnetic waves whose wave have length is less than 3000  $\text{\AA}$  can also be used. The exposure can be carried out by means of a mercury lamp or the like, e.g., xenon lamp etc. The exposed material is then uniformly heated to a temperature of from room temperature to about 200°C. In general, heating is for from several seconds to 20 minutes, with standard heating being for 30 seconds - 5 minutes at 100°C or so for superior printing plate formation. The heating may be carried out with 2.5-20  $\mu$  infrared irradiation.

In the printing plate embodiment, images which are distinguishable are then treated with a solvent in order to remove parts unnecessary in the printing plate (namely, non-printing or unexposed parts) so as to expose the hydrophilic surface of the support. The solvent used can be suitably selected on the basis of the binder used. The solvents used include, for example, alcohols, preferably C<sub>1</sub>-C<sub>10</sub> alcohols, such as methanol, ethanol, propanol, butanol, cyclohexyl alcohol and ethylene glycol, ketones, preferably C<sub>1</sub>-C<sub>8</sub> ketones, such as acetone, methylethyl ketone and cyclohexanone, aromatic solvents, preferably C<sub>6</sub>-C<sub>10</sub> aromatic solvents, such as benzene, toluene and xylene, ethers, preferably C<sub>2</sub>-C<sub>6</sub> ethers, such as diethyl ether, dioxane and tetrahydrofuran, and esters, preferably C<sub>3</sub>-C<sub>15</sub> esters, such as ethyl acetate, ethyl formate and  $\gamma$ -butyrolactone.

Good results are obtained at the following solvent treatment conditions: temperature, ca. 30° to ca. 200°C, preferably 50°-150°C, time, ca. 2-3 sec. to ca. 10 min., preferably 30 sec.- 5 min., pressure, 1 atm., though sub or super atmospheric pressures can be used.

According to the present invention, good printing plates having excellent printing durability can be produced by exposure to light, heating and solvent treatment. Further, since visible images resulting during production of the printing plate, inspection of the printing plate can be easily carried out.

In the present invention, the used furfurylidene compound is quite stable, and thus the resulting photosensitive materials are excellent in preservability for a long period of time, and moreover, an image with less background stain can be formed. Furthermore, a permanent image can be obtained, as the case may be, only by the operation combined with the heating step, and the obtained image has excellent properties such as high weather resistance, high chemical resistance and the like, that is, any bleeding or fading does not occur in the image. Thus, the photo-sensitive materials of the present invention have various merits which could not be attained in the conventional photo-sensitive materials for forming colored images.

Now, the present invention will be explained more in detail in the following examples where: Examples 1-5 deal with the non-silver salt photosensitive material per se and Examples 6-15 deal the printing plate embodiment.

In the Examples, all percentages are by weight, unless otherwise indicated.

#### EXAMPLE 1

After 0.1g of difurfurylidene-pentaerythritol and 0.1g of iodoform were dissolved in 3g of a 5% polystyrene-benzene (polystyrene of an average polymeri-

zation degree of about 900) solution, the resulting solution was applied to a photographic baryta paper using a coating rod, and then dried for 30 minutes in a drying chamber at 70°C to prepare a light-sensitive material (light sensitive layer: ca 3  $\mu$  thick).

The thus prepared light-sensitive material was contacted with a negative film, and exposed for 20 seconds by means of a diazotype duplicator with a built-in 600W mercury-vapor lamp at 20 cm. distance, whereby a yellow image was obtained (main wavelength: 3650 Å).

Next, the material was heated for 120 seconds at 120°C to obtain a brown image having a reflection density of 1.35. The background of the material was colorless. When the material was exposed to sun-light for one day, the background colored yellow while the image was unchanged.

#### EXAMPLE 2

0.1g of difurfurylidene-pentaerythritol, 0.1g of carbon tetrabromide and 0.1g of phloroglucinol were dissolved in 3g of a 5% polystyrene-tetrahydrofuran (polystyrene of an average polymerization degree of about 900) solution, and the resulting solution was applied to a photographic baryta paper using a coating rod and then dried for 15 minutes in a drying chamber at 50°C (light sensitive layer ca. 3  $\mu$  thick).

The resulting light-sensitive paper was closely contacted with a negative film, and exposed for 20 seconds by a diazotype duplicator with a built-in 600W mercury-vapor lamp 20 cm from the element, whereby a positive image colored a strong dark green color was obtained. The reflection density of the formed image was 1.41.

Next, the paper was heated for 30 seconds at 110°C, whereby the color of the image changed to blackish, and the reflection density thereof increased to 1.86. There was no stain in the background of the paper.

When the material was left in a light room without exposure to direct sun light, the color did not change and the background was not stained.

When the material was continuously exposed to direct sun-light for one week, the color image was not changed, but the background somewhat colored pale brown.

Separately from the above, the light-sensitive paper prepared as above herein was exposed using a Uniarc 250-60 (manufacturer: Ushio Electric Co. main wavelength: 3650 Å) with a built-in 250W super high pressure mercury vapor lamp (a light source for IC printing) at a distance of 40 cm from the shutter thereof and then heated with a hot plate at 110°C. The color density of the resulting image is shown in the following Table.

|                             |      |      |      |      |
|-----------------------------|------|------|------|------|
| Time for exposure (seconds) | 100  | 50   | 25   | 12.5 |
| Time for heating (seconds)  | 10   | 10   | 10   | 10   |
| Optical density             | 0.99 | 0.75 | 0.61 | 0.33 |

#### EXAMPLE 3

0.1g of difurfurylidene pentaerythritol, 0.1g of iodoform, 0.1g of pyrogallol and 3g of a 10% polyvinyl butyral-tetrahydrofuran (polyvinyl butyral: about 700 average polymerization degree) solution were coated to prepare a light-sensitive paper (3  $\mu$  thick light sensitive layer), and the resulting paper was exposed, as in Example 2, whereby an image of orange color was formed on a background of a pale-yellow color. The resulting paper was heated for 30 seconds at 100°C, whereby the color of the image changed to a dark black-brown color.

Separately, a light-sensitive paper prepared as above except using only 0.1g of iodoform and 0.1g of pyrogallol was exposed to light. Although an image of orange color was obtained, the color of the resulting image faded to a pale yellow color after heating under the same conditions as above.

#### EXAMPLE 4

0.1g of furfurylidene acetal, 0.1g of a haloalkane and 0.1g of a phenol type compound were dissolved in 10% resin solution, as identified in the following Table. The resulting solution was applied to a baryta coated paper and dried to provide a light sensitive layer 4  $\mu$  thick as in Example 2. The thus prepared light-sensitive material was exposed and heated as in Example 2.

| furfurylidene compound                                    | haloalkane          | phenol type compound         | high molecular weight binder (resin) | color           |
|-----------------------------------------------------------|---------------------|------------------------------|--------------------------------------|-----------------|
| difurfurylidene-pentaerythritol                           | carbon tetrabromide | gallic acid                  | polystyrene*                         | brown           |
| "                                                         | "                   | n-ethyl gallate              | "                                    | olive brown     |
| "                                                         | "                   | 1,5-dihydroxy-naphthalene    | "                                    | yellowish-brown |
| "                                                         | iodoform            | 2,4,6-dihydroxy-acetophenone | polyvinyl-butyral**                  | dark green      |
| "                                                         | "                   | 2,4,6-dihydroxy-toluene      | "                                    | dark green      |
| furfurylidene-2-ethyl-2-hydroxymethyl-1,3-propylene ether | carbon tetrabromide | phloroglucinol               | polystyrene*                         | dark green      |
| furfurylidene-furfuryl alcohol                            | "                   | phloroglucinol               | "                                    | black           |

| furfurylidene compound                                           | haloalkane | phenol type compound | high molecular weight binder (resin) | color      |
|------------------------------------------------------------------|------------|----------------------|--------------------------------------|------------|
| furfurylidene-2-methyl-2-furfurylidene-imino-1,3-propylene ether | "          | phloroglucinol       | "                                    | dark green |
| furfurylidene-diphenyl ether                                     | "          | pyrogallol           | "                                    | brown      |

\*average polymerization degree about 900

\*\*average polymerization degree about 700

## EXAMPLE 5

0.1g of difurfurylidene-pentaerythritol, 0.1g of carbon tetrabromide and 0.1g of a phenol type compound were dissolved in a 5% polystyrene-tetrahydrofuran solution (same as Example 2) and treated as in Example 2 to obtain a light-sensitive material. The material was exposed to light for 30 seconds using a 600W diazotype duplicator 20 cm from the material (main wavelength 3650 Å) to form a visible latent image colored pale brown. After heating for 60 seconds at 110°C. a brown image having a reflection density of 0.5-0.9 was obtained. The phenol type compound added to the light-sensitive material to form a series of different elements was as follows: methyl gallate, propyl gallate, isoamyl gallate, lauryl gallate, 3-methoxy-catechol, catechol, 2,5-dihydroxy-benzoic acid, 3,4-dihydroxy-benzoic acid, 2,4-dihydroxy-5-bromobenzoic acid, 2,6-dihydroxy-benzaldehyde or p-hydroxy-benzene-sulfonic acid.

## EXAMPLE 6

A printing plate making material was prepared by dissolving 0.1g of carbon tetrachloride, 0.1g of difurfurylidene pentaerythritol and 0.1g of phloroglucinol in 3g of a 5% tetrahydrofuran solution of polyvinyl butyral (Eslex BM 5, Sekisui Kagaku), and applying the resulting solution to an anodized aluminum plate. The thickness of the photosensitive layer was 2 μ. The anodization conditions were: 40% phosphoric acid, room temperature, 10 A/cm<sup>2</sup> electric current supplied for 2 minutes. This is a conventional art procedure.

A negative film was brought into physical contact with the resulting plate making material. The printing plate making material was then exposed to light from a 600W mercury lamp at a 20 cm distance through a plexy filter for 20 seconds whereupon a positive printing-out image was formed.

This printing plate making material was then heated for one minute on a heating plate at 110°C, whereupon the positive printing-out image changed to a dark brown color image. By washing with methanol at room temperature for 1 minute, unexposed parts were removed, i.e., peeled off. Upon further washing with water, a printing plate for negative working was obtained, in which the exposed parts remained as a brown image.

Though this printing plate could be utilized as it was on a printer, it was possible to increase the oleophilic property of the image part and to improve the abrasion resistance by applying a lacquer thereto. Further, the hydrophilic property of the non-image part was improved by a rubbering treatment.

## EXAMPLE 7

A printing plate making material was produced by dissolving 0.1g of carbon tetrabromide, 0.2g of difurfurylidene pentaerythritol and 0.6g of phloroglucinol in 9g of a 5% tetrahydrofuran solution of polyvinyl butyral (Eslex BM 5, Sekisui Kagaku), and applying the resulting solution to an anodized aluminum plate. The thickness of the photosensitive layer was in the range 1-4 μ.

After putting a positive film on the resulting printing plate making material, it was exposed to light in the same manner as in Example 6 and treated by heating at 110°C for 2 minutes. A deep dark-green image appeared on the surface of the printing plate making material.

The printing plate material was then washed with ethyl alcohol at room temperature for 2 minutes and then with water at room temperature for 2 minutes. A printing plate for positive working was thus obtained.

Further, the printing plate was treated with a development ink in order to improve the oleophilic property of the image parts, whereby a positive image was formed. When the plate was subjected to rubbering treatment, the hydrophilic property of the non-image parts was further improved.

## EXAMPLE 8

A printing plate making material was produced by dissolving 0.1g of carbon tetrabromide, 0.1g of difurfurylidene pentaerythritol and 0.1g of 4-ethylresorcinol in 3g of a 5% tetrahydrofuran solution of polymethyl methacrylate, and applying the resulting solution to the same support and in the same manner as in Example 6. The thickness of the photosensitive layer was in the range 1-4 μ.

A printing plate for positive working was produced by exposure to light in the same manner as in Example 7, carrying out heat treatment (110°C) for 30 seconds, and treating thereafter in the same manner as in Example 7.

## EXAMPLE 9

Printing plate making materials were produced by dissolving 0.1g of carbon tetrabromide, 0.1g of one of the following furfurylidene acetal compounds and 0.1g of one of the following phenolic compounds in a 5% tetrahydrofuran solution of polyvinyl alcohol (Sebian A-235, Daisel Co., Ltd) and applying the resulting solutions to the same support and in the same manner as in Example 1. The thickness of the photosensitive layer was in the range 1-4 μ.

Positive printing plates for positive working were produced by exposing to light in the same manner as in

Example 7, carrying out heat treatment at 110°C for a period as described in the following table, and then unexposed areas removed with solvent (plate making treatment).

| Phenolic compound             | Furfurylidene acetal compound                                   | Heating time (seconds) |
|-------------------------------|-----------------------------------------------------------------|------------------------|
| Catechol                      | Difurfurylidene pentaerythritol                                 | 120                    |
| Catechol                      | Furfurylidene 2-methyl-2-furfurylideneimino-1,3-propylene ether | 120                    |
| Pyrogallol                    | Difurfurylidene pentaerythritol                                 | 60                     |
| Hydroquinone                  | Difurfurylidene pentaerythritol                                 | 120                    |
| 4-Bromoresorcinal             | Difurfurylidene pentaerythritol                                 | 30                     |
| 4,6-Dichlororesorcinal        | Difurfurylidene pentaerythritol                                 | 60                     |
| 5-Methylresorcinol            | Difurfurylidene pentaerythritol                                 | 90                     |
| 5-Methylresorcinol            | Furfurylidene 2-ethyl-2-hydroxymethyl-1,3-propylene ether       | 60                     |
| 2-Methylresorcinol            | Difurfurylidene pentaerythritol                                 | 40                     |
| Resorcinol                    | Difurfurylidene pentaerythritol                                 | 30                     |
| Resorcinol                    | Furfurylidene bis-(p-chlorobenzyl ether)                        | 60                     |
| 2-Aminophenol                 | Difurfurylidene pentaerythritol                                 | 180                    |
| 1,3-Dihydroxy-naphthalene     | Difurfurylidene pentaerythritol                                 | 30                     |
| 4-Methoxy- $\alpha$ -naphthol | Difurfurylidene pentaerythritol                                 | 60                     |
| 2,4,6-Trihydroxytoluene       | Difurfurylidene pentaerythritol                                 | 60                     |
| 2,4,6-Trihydroxyacetophenone  | Furfurylidene dianisyl ether                                    | 60                     |

#### EXAMPLE 10

A printing plate making material was produced by dissolving 0.1g of carbon tetrabromide, 0.1g of difurfurylidene pentaerythritol and 0.3g of phloroglucinol in 4g of a 5% ethyl acetate solution of cellulose acetate butyrate and applying the resulting solution to an anodized aluminum plate in the same manner as in Example 6. The thickness of the photosensitive layer was in the range 1-4  $\mu$ .

The printing plate making material was exposed to light in the same manner as in Example 7, heated at 110°C and washed with a solution of ethyl alcohol-acetone (2:1 by volume) at 25°C for 3 minutes and then with water at 25°C for 30 minutes. The plate was then treated in the same plate making treatment as in Example 6, by which a printing plate for positive working was produced.

#### EXAMPLE 11

A printing plate making material was produced by dissolving 0.1g of carbon tetrabromide, 0.1g of difurfurylidene pentaerythritol and 0.1g of phloroglucinol in a 5% tetrahydrofuran solution of polyvinyl formal (Denka Formal 3000, Denki Kagaku Kogyo Co., Ltd.) and applying the resulting solution to an anodized aluminum plate in the same manner as in Example 6. This printing plate making material was exposed to light in the same manner as in Example 7, heated at 60°C for 5 minutes, washed once with ethyl alcohol at 40°C for 2 minutes, and then washed with water at 25°C for 1

minute, whereupon a printing plate for positive working was produced. The thickness of the photo sensitive layer was in the range 1-4  $\mu$ .

#### EXAMPLE 12

5 A printing plate making material was produced by dissolving 0.1g of iodoform, 0.1g of difurfurylidene pentaerythritol and 0.3g of phloroglucinol in a 5% tetrahydrofuran solution of polyvinyl acetate and applying 10 the resulting solution to an anodized aluminum plate in the same manner as in Example 6. The thickness of the photosensitive layer was in the range 1-4  $\mu$ .

A printing plate for positive working was produced 15 by exposing to light, heating and washing in the same manner as in Example 7.

#### EXAMPLE 13

A printing plate making material was produced by 20 dissolving 0.1g of carbon tetrabromide, 0.1g of 2,5-dihydroxy-benzoic acid and 0.1g of difurfurylidene pentaerythritol in a 5% tetrahydrofuran solution of polyvinyl butyral (same as in Example 6) and applying the resulting solution to an anodized aluminum plate in the same manner as in Example 6. A printing plate for negative working was produced by exposing to light in the same manner as described in Example 6, applying heat by means of a 500 watt infrared ray lamp at 15 cm distance for 4 minutes, and then carrying out the plate making treatment in the same manner as in Example 6. 30 The thickness of the photosensitive layer was in the range 1-4  $\mu$ .

#### EXAMPLE 14

A printing plate making material was produced using 35 0.1g of  $\alpha,\alpha,\alpha$ -p-tetrabromoacetophenone, 0.1g of difurfurylidene pentaerythritol and 0.1g of phloroglucinol in the same manner as in Example 6. This printing plate making material was exposed to light, heated and treated with solvent in the same manner as in Example 6 to produce a printing plate for positive working. The thickness of the photosensitive layer was in the range 1-4  $\mu$ .

#### EXAMPLE 15

45 A printing plate making material was produced by dissolving 0.2g of  $\alpha,\alpha,\alpha$ -tetrabromoacetophenone, 0.1g of difurfurylidene pentaerythritol and 0.06g of phloroglucinol in a 5% tetrahydrofuran solution of polyvinyl butyral (same as in Example 6), applying the resulting 50 solution to an aluminum plate the surface of which was grained, and drying. The thickness of the photo-sensitive layer was in the range 1-4  $\mu$ . This printing plate making material was exposed, heated and treated with solvent in the same manner as in Example 6 to produce a printing plate for negative working.

#### EXAMPLE 16

A printing plate making material was produced by 60 dissolving 0.1g of  $\alpha,\alpha,\alpha$ -tribromomethylphenylsulfone, 0.1g of furfurylidene 2-ethyl-2-hydroxymethyl-1,3-propylene ether and 0.1g of phloroglucinol in a 5% tetrahydrofuran solution of polyvinyl butyral, and then treating in the same manner as in Example 6. The thickness of the photosensitive layer was in the range 65 1-4  $\mu$ . The printing plate making material was then exposed to light, heated and treated with solvent in order to produce a printing plate for positive working.

Thus, from the above it is seen that the haloalkane and phenol compound react together by exposure, and a great amount of halogenic hydrogen is formed. The thus formed halogenic hydrogen is used as a catalyst, e.g., ring opening polymerization of the furfurylidene, and acid polycondensation of the phenolic compound and the hydrolysis product of furfurylidene, etc., proceeds. Uniform heating shortens the reaction time of the above.

While the invention has been described in detail and with reference to specific embodiments thereof, it will be apparent to one skilled in the art that various changes and modifications can be made therein without departing from the spirit and scope thereof.

What is claimed is:

1. Non-silver salt photo-sensitive materials which consist essentially of a light-sensitive layer containing as image-forming components a high-sensitive haloalkane having a dissociation energy of less than 75 Kcal/mol, a furfurylidene acetal compound of the following formula (IIa) or formula (IIb):



wherein R<sub>1</sub> and R<sub>2</sub> each represents one or two phenyl groups or one or two aralkyl groups, or one or two furyl groups;



wherein R<sub>3</sub> represents an alkylene group having 2-7 carbon atoms, which can be substituted with a hydroxyl group having 1-4 carbon atoms or an amino group, or may be dimerized by a spiro carbon, and a phenol compound of formulae (IIIa) or (IIIb)



wherein n is an integer of 1-3, and R<sub>4</sub> represents a hydrogen atom, a halogen atom, an alkyl group of 1-4

carbon atoms, an alkoxy group of 1-4 carbon atoms, a carboxyl group, an alkoxycarbonyl group of 1-12 carbon atoms, a formyl group, a sulfo group or an acyl group of 1-4 carbon atoms.

5. Non-silver salt photo-sensitive material as claimed in claim 1 where the haloalkane is of the formula



(I)

10 wherein X represents a halogen atom (where X's may differ from each other) or a hydrogen atom (but all X's cannot be hydrogen atoms), and R represents a hydrogen atom; a halogen atom; an alkyl group having 1-7

15 carbon atoms; a halogen substituted alkyl group having 1-7 carbon atoms; an acyl group; or an acyl group or arylsulfonyl group substituted with a halogen atom, a nitro group or an aryl group.

20 3. Non-silver salt photo-sensitive materials as claimed in claim 1 wherein said haloalkane is carbon tetrabromide, iodoform, carbon tetraiodide, hexachloroethane, hexafluoroethane, 1,2-diiodoethane, bromotriiodomethane or chloro-diiodomethane.

25 4. Non-silver salt photo-sensitive materials as claimed in claim 1 wherein said furfurylidene acetal is difurfurylidene pentaerythritol, furfurylidene 2-ethyl-2-hydroxymethyl-1,3-propylene-ether, furfurylidene difurfuryl-ether, furfurylidene-2-methyl-2-furfurylideneimino-1,3-propylene-ether, furfurylidene-30 tetramethylene-ether, furfurylidene-diphenethyl-ether, furfurylidene-dibenzyl-ether, furfurylidene-dianisyl-ether, furfurylidene-dibenzohydrylether or furfurylidene-bis-(p-chlorobenzylether).

35 5. Non-silver salt photo-sensitive materials as claimed in claim 1 wherein said phenol compound is pyrogallol, methyl gallate, ethyl gallate, n-propyl gallate, isoamyl gallate, lauryl gallate, stearyl gallate, gallic acid, phloroglucinol, 2,4,6-trihydroxy-toluene, 2,4,6-trihydroxy-acetophenone, 3-methoxy-catechol, 2,3,4-dihydroxy-benzoic acid, 2,5-dihydroxy-benzoic acid, 2,6-dihydroxy-3,5-di-tert.butyl-benzoic acid, 2,6-dihydroxy-benzaldehyde, 4,5-dihydroxy-toluene, resorcinol, 4-chloro-resorcinol, 3,5-dihydroxy-toluene, hydroquinone, p-hydroxybenzene-sulfonic acid, p-bromophenol, 1,5-dihydroxy-naphthalene, 1,3-dihydroxy-naphthalene or 2,7-dihydroxy-naphthalene-3-sulfonic acid.

40 6. Non-silver salt photo-sensitive materials as claimed in claim 1 wherein the said light-sensitive layer additionally contains a film forming binder.

45 7. Non-silver salt photo-sensitive materials as claimed in claim 6 where the binder is nitrocellulose, benzyl cellulose, polycarbonate, polyvinyl acetate, cellulose acetate, cellulose acetate butyrate, cellulose acetate phthalate, polyvinyl chloride, polystyrene, polyester, polymethyl methacrylate, polyvinyl pyrrolidone, polyvinyl butyral or polyphenyleneoxide.

50 8. Non-silver salt photo-sensitive materials as claimed in claim 1 where the weight ratio of the haloalkane to the furfurylidene acetal is 0.1-3.

55 9. Non-silver salt photo-sensitive materials as claimed in claim 8 where the weight ratio is 0.5-2.

10. Non-silver salt photo-sensitive materials as claimed in claim 1 wherein the weight ratio of the phenol compound to the furfurylidene acetal is 5 or less.

60 11. Non-silver salt photo-sensitive materials as claimed in claim 10 where the weight ratio is 0.05-2.

12. Non-silver salt photo-sensitive materials as claimed in claim 1 wherein said light-sensitive halo-alkane has the following formula (I):



(1)

5 wherein each X may be same or different and represents a halogen atom or hydrogen atom, but every X cannot be a hydrogen atom, and R represents a hydro-

gen atom, a halogen atom or a halogen-substituted alkyl group having 1-3 carbon atoms.

\* \* \* \* \*

10

15

20

25

30

35

40

45

50

55

60

65